

## UNITED STATES PATENT OFFICE

JOHANN JOSEPH STÖCKLY, OF TELTOW, AND ERHARD WITTE, OF BERLIN-LICHTER-FIELDS, GERMANY, ASSIGNS, BY MESNE ASSIGNMENTS, TO AMERICAN GLANZ-STOFF CORPORATION, OF NEW YORK, N. Y.

## ARTIFICIAL SILK

No Drawing. Application filed April 9, 1929, Serial No. 353,889, and in Germany October 2, 1928.

It is known that products of artificial silk, especially fibres and threads, have been rendered opaque or mat by incorporating certain organic substances in the spinning substance, and especially with viscose silk it is known to incorporate for this purpose in the viscose liquid emulsifiable substances, such as petroleum.

According to the present invention for making products of viscose, for instance artificial viscose silk, opaque or mat, such substances are best suited which are particularly insoluble in water, and which will remain solid at ordinary temperatures, and will not be practically changed by the alkali of the viscose or by the acid of the spinning bath, said substances not being emulsifiable per se in the viscose, but they will become dissolved by suitable organic substances.

Such substances are, for example, waxes, for instance Japan wax, mineral wax, or paraffine, or ozokerite, and beeswax.

According to this invention these waxes are dissolved in suitable organic substances such as benzol, toluol, xylol or mixtures thereof, and the solution emulsified with the viscose.

This can be done by adding such a solution of a wax to the viscose, for example in the mixer when dissolving the xanthates, or by adding them to the finished viscose in an efficient emulsifying machine. The viscose is then filtered and spun under the customary precautions.

The process permits adding variable quantities of these normally solid or semi-solid waxes, to obtain various degrees of the mat effect of the products of the viscose, especially on viscose threads.

According to the character or kind of the substance and the degree of mat desired, a larger or smaller quantity of the solid wax is added, and in accordance with this the quantity of the organic solvent is also defined.

The said waxes are especially adaptable for artificial threads, because they are incorporated within the body of the thread during the spinning process. In this way this invention is distinguished from the

usual finishing process, wherein the threads are loaded with wax after they are made, and then on the exterior of the thread only.

## Example 1

55

To 100 kilograms of normal viscose in a mixer is added a solution of 400 grams of Japan wax dissolved in 900 grams of benzol, and the mixture well emulsified. The product is then filtered and de-aerated, and after proper ripening in the usual manner, is spun in the customary way.

## Example 2

65

To 100 kilos of normal viscose is added a solution of 500 grams of ozokerite dissolved in 1500 grams of benzol, and the mixture well emulsified; the resultant viscose solution is then treated in the customary way and spun.

For beeswax xylol is the preferred solvent. The emulsion and spinning are as above described.

We claim:

As a solution for use in the manufacture of dull lustre filaments, threads, bands, and the like, a filtered and deaerated mixture comprising:

|                | Per cent |
|----------------|----------|
| Viscose-----   | 98.7 80  |
| Japan wax----- | 0.4      |
| Benzol-----    | 0.9      |

In testimony that we claim the foregoing as our invention, we have signed our names 85 hereto.

JOHANN JOSEPH STÖCKLY.  
ERHARD WITTE.

90

95

100